

## UNITED STATES PATENT OFFICE

ARTHUR HOUGH, OF SUMMIT, JOHN ROY DUFFORD, OF PATERSON, AND WILLIAM CLELLAND LEONARD, OF PASSAIC, NEW JERSEY

## MANUFACTURE OF NITROCELLULOSE

No Drawing.

Application filed August 31, 1926. Serial No. 132,906.

Our invention relates to improvements in nitrated products and also involves the mode of preparation of a relatively cheap, exceedingly stable nitrated product, very soluble in those solvents commercially employed in the manufacture of celluloid, lacquers, and kindred products. It may also be used in the preparation of smokeless powders or propellants in the explosive industry wherein such nitrated material can be advantageously employed.

To carry out the invention, vegetable parchment is first made by any of the well-known methods, such as treatment of cellulose as such or the more impure type known as wood pulp or preferably alpha fibre pulp by sulphuric acid of the desired strength, or any suitable parchmentizing reagent.

The preferred mode of parchmentizing the sheets (commonly called "waterleaf", which is an unsized paper, of any desired thickness) is the usual and customary method which comprises immersing the paper, for a short time (a few seconds up to a minute or two) in sulphuric acid of between 54° Bé. and 56.5° Bé. (68.6% to 72.4%) and preferably between 55° Bé. and 55.5° Bé. (70% and 70.85%), the acid being cold, say at below 60° F., and preferably at not above 50° F. The paper is then removed from the acid bath and washed with water, while being kept cold. Under these conditions, which are those always used in commercial parchmentizing, no dextrinization of the cellulose occurs.

The sheets, which are usually of about 23 to 25 lbs., thickness, are sufficiently porous so that the parchmentizing acid and the nitrating acid readily penetrate the sheets, and both the parchmentizing and the nitrating steps are substantially complete. The parchmentized material is then comminuted into pieces of the desired size, and on account of the fact that the paper is parchmentized, there is no loose fibers or dust on the pieces of parchmentized paper. The comminuted parchmentized paper is then soaked in the nitrating acids for sufficient time to insure complete nitration and at a temperature approximating 40° C. if maxi-

mum solubility in the selected solvent is required.

This nitration is preferably effected by treating this parchment in a mixture of H<sub>2</sub>SO<sub>4</sub> plus HNO<sub>3</sub> plus H<sub>2</sub>O; the ratio of one acid to the other and to the water content depending upon the degree of nitration desired as also the degree of solubility looked for in the selected solvents. For example if nitrated parchment of about 11% nitrogen content is required, with an extremely high solubility of the product in camphor-alcohol mixture, then the acid mixture may be close to 60% H<sub>2</sub>SO<sub>4</sub>; 21% or 22% HNO<sub>3</sub>; and 18% or 19% H<sub>2</sub>O. The temperature of the acids during nitration may be about 40° C. Under these conditions no dextrinization can occur.

At a lower temperature, the time of nitration is longer, and the solubility of the product is somewhat less. We do not, however, confine ourselves to this acid mixture or temperature and we may vary them somewhat depending upon the properties desired, in the finished product.

The nitration having been completed, the spent acid, so called, is now removed and the product washed with ordinary water till the degree of acidity has been reduced to approximately 1%. On account of the freedom from loose fibers and dust, the waste nitrating acid which drains off from the nitrated parchment does not carry small bits of cellulosic material, hence the usual difficulties attending the regenerating of the nitrating acids from gun cotton and from nitrated wood pulp, are avoided. The nitrated parchment is now boiled in excess of water for about three hours, when the water is removed, the product washed free from acid and fresh water added, to which is added sufficient ammonium hydroxide, or its equivalent, to render the water just alkaline (slightly alkaline) to litmus. Heating should continue for about two or three hours or longer. At this point it will be seen that the water is colored strongly yellow, due to the decomposition of the nitrated impurities in the parchment that must be removed to render the product stable, since retention in

the product would make the same unstable. In these subsequent treatments with ammonia, the ammonia must be added cautiously, preferably only enough ammonia to make the water alkaline to phenolphthalein. Any larger excess of ammonia would injure the product. Repeated renewal of water and very slight additions of ammonia hydroxide, or its equivalent, must be made till no more 5 yellow color, or very little develops on heating and the check samples taken from the heater show the required stability test with potassium iodide starch paper, the stability test at 135° C., and the flash point between 10 170° C., and 180° C.

When this point has been reached, the product may be bleached if desired. In order to preserve the original stability an alkaline bleach must be employed, an acid bleach 20 would impair the stability of the product. A suitable bleaching agent is an alkaline sodium hypochlorite liquor, the quantity of such bleach to be used will depend upon the speed desired in bleaching, and this matter 25 must be left to the discretion of the operator.

Having described the invention, we claim:

1. A nitrated product prepared from parchmentized paper stabilized by treatment with hot dilute ammonium hydroxide and 30 bleached with an alkaline bleach, substantially as described.

2. A nitrated product prepared from material consisting essentially of vegetable parchment having as the basic substance nitrated parchmentized sheeted wood pulp, substantially free from matter which would dissolve in very dilute boiling ammonia water and which matter when so dissolving in dilute ammonia would produce a strong yellow color, such nitrated parchment also having excellent stability as shown by the usual 40 nitrocellulose tests.

3. The process of making a nitrated product by parchmentizing sheeted wood pulp 45 with sulphuric acid, washing the parchment substantially free from acid, then drying same and nitrating the dry pulp in the form of comminuted parchmentized paper in a nitration mixture, and dissolving out nitrated impurities, substantially as described.

4. The process of making a nitrated product by subjecting sheeted alpha fibre pulp to parchmentizing in sulphuric acid, under parchmentizing but not dextrinizing conditions, washing the parchmentized product substantially free from acid, then drying same and nitrating the parchmentized product in the form of "waterleaf" in a nitration acid mixture containing  $H_2SO_4$  and 55  $HNO_3$ , washing acid-free, and dissolving out nitration products soluble in very dilute ammonia water, substantially as described.

5. A process of treating wood pulp which 60 comprises treating said pulp in the form of "waterleaf" with sulphuric acid to parch-

mentize the pulp, washing the pulp to a substantially acid-free condition, nitrating the parchmentized waterleaf with a mixture of sulphuric and nitric acids, washing the pulp with water to remove the free acid, and heating the nitrated product with water containing a small percentage only of ammonia so as to remove nitrated products of impurities without altering the pure nitrated waterleaf, and continuing such treatment until the ammonia 70 wash water remains nearly clear.

6. A process which comprises parchmentizing paper, and thereafter nitrating the parchmentized paper, by treatment with mixed nitric and sulphuric acids.

7. A process which comprises parchmentizing paper, thereafter nitrating the parchmentized paper, thereafter washing well with water to remove all free acid, and thereafter boiling the product with water 85 containing a small amount of ammonia.

8. Nitrated paper parchment, in a substantially stable condition.

ARTHUR HOUGH.

JOHN ROY DUFFORD.

WILLIAM CLELLAND LEONHARD.

75

75

80

85

90

95

100

105

110

115

120

125

130